

Feb. 8, 1944.

C. D. COXE

2,341,264

AMMUNITION

Filed June 12, 1940

Fig. 1



A

Fig. 3



Fig. 2



INVENTOR  
Charles D. Coxe

BY

*Donald S. Smith*  
ATTORNEYS

## UNITED STATES PATENT OFFICE

2,341,264

## AMMUNITION

Charles D. Coxe, Bridgeport, Conn., assignor to  
Remington Arms Company, Inc., a corporation  
of Delaware

Application June 12, 1940, Serial No. 340,003

3 Claims. (Cl. 148—12)

This invention relates to the manufacture of ammunition components from steel. Brass and gilding metal are the commonly used components for ammunition, particularly the cases, because they are the only metals previous to the invention described herein that have satisfactorily met the requirements of ammunition components in regard to cost, shaping, strength, corrosion resistance and extractability from the gun. Brass, however, has many disadvantages, and among them may be enumerated cost, tendency to season crack, and the tendency to react or cause the primers and/or powder contained therein to become unstable. Gilding metal is expensive as compared to steel. In the embodiment disclosed, the use of steel is shown as applied to a cartridge case and also for other of the ammunition components such as, for example, shot shell heads and center fire primer cups. In the use of metals for a cartridge case, it has been found that the metal must have a sufficiently high yield strength so that the case will not bulge under theurgence of the powder pressures and appreciably remain in the bulged condition, thereby preventing extraction of the case from the chamber of the gun. It is also necessary that the metal be sufficiently ductile and in such a condition that splits will not occur near the mouth of the case upon firing of the cartridge. Gilding metal has been found to work satisfactorily in the standard loads and to give the desired results. There have been many attempts to use steel but such has never proven feasible. The other objects of the invention will appear from the following description and illustrations which, as stated before, are not intended to limit the invention to the form shown and described.

In the drawing:

Fig. 1 is a sectional view of a rimfire cartridge case after it has been fired in the chamber of a gun wherein the clearance between the case and the chamber of the gun is shown exaggerated. The bulging of the shell due to firing pressures and a split in the case are also shown in exaggerated form.

Fig. 2 shows diagrammatically, by way of example, sectional views of five stages in the forming of a rimfire shell from a flat blank to the finished rimfire case.

Fig. 3 is a graph showing the percentage of splits and extraction force required for various cartridge cases treated in various manners.

The conventional gun is provided with a chamber into which the cartridge case fits, the clear-

ance between the cartridge case and the chamber being governed by many factors. The cartridge case is properly sized in the course of manufacture to fit into the chamber, but the fit will vary 5 due to manufacturing tolerances of the cases as well as the tolerances in the machining of the chamber of the gun. Also the roughness or smoothness of the chamber of the gun will affect the operation and extraction of the case from the 10 chamber. As the cartridge is fired, the pressure of the powder gas forces the projectile through the barrel of the gun, and, at the same time, the cartridge case is forced radially outwardly to fill the clearance substantially completely, thereby 15 sealing the powder gases and preventing the escape thereof backward through the working mechanism of the gun instead of acting to force the projectile through the barrel. It is evident from this that the metal of the case must have sufficient resilience to return into its original condition 20 so that the case may be extracted from the gun after firing the shell. The yield strength must not have been passed appreciably in this preceding action, for otherwise the case will stay, 25 at least partially, in its bulged condition and prevent satisfactory extraction. The yield point may be defined as the point before which no plastic deformation takes place. The metal of the case must also be in such a condition that 30 there will be sufficient ductility so that the case will not split upon firing. Referring to Fig. 1, there is shown a conventional rimfire shell in which 10 represents the bolt of the gun which has been closed on the head 11 of the case 12, 35 the case 12 fitting within the chamber 13 of the barrel 14 of the gun. Extractor 15 of a conventional type engages the rim of the shell so that as the bolt is withdrawn or operated, the shell will be removed from the chamber. The usual 40 striker or firing pin 22 is provided to strike the rim of the case 12 wherein the priming mixture is located. In the illustration, the section is across the receiver, and it is to be noted that the point of contact of the striker and the shell 45 is at or near the edge of the rim of the shell. If the yield point has been exceeded, the case will remain bulged outwardly, for example, as seen in exaggerated form at 16 of Fig. 1, and splits will occur, as at 17, if there is insufficient ductility or the grain structure of the metal is such 50 as not to allow the stretching of the metal as the propellant charge is ignited. In the manufacture of cartridges and ammunition, particularly of the smaller calibers, it is the usual practice to employ charges and powders giving dif-

ferent velocities. These may be classified generally as the high velocity and low or standard velocity. In order to obtain the high velocity, it is necessary that a larger powder charge be used or a charge be employed which will develop higher pressure or characteristics to force the projectile outwardly through the barrel at the desired velocity. In the conventional .22 caliber long rimfire shells, the high velocity bullets leave the gun at about a velocity of 1375 feet per second, and powder pressure developed within the barrel is in the neighborhood of 18,000 pounds per square inch. This is in contrast to the standard of lower velocity cartridges, wherein the velocity may be in the neighborhood of 1030 feet per second, with a powder pressure developed in the barrel of 14,000 pounds per square inch. By the invention herein described, it has been found possible to use steel, relief annealed, in place of brass or gilding metal for both high and standard velocities. It is necessary in the selection of the metal to be used that due regard be given to using a metal that will properly draw in the manufacture of the cartridge case or component.

In Fig. 2, A, B, C, D, E, are shown some of the steps in the drawing of a conventional rimfire shell, although, as previously stated, the invention is not limited to the type and form shown, and the number and form of operations may vary. In A is seen a cross section of a flat blank, and B is the same blank after it has been cupped, the usual practice being for the blank A to be cut from a strip and cupped by the same punch. C, D and E show the succession of forms as the cup B is drawn through the various dies and finally headed at E. When the case is in the form shown in E, it is not satisfactory for use as a cartridge case, and must be properly heat treated to give the desired results.

The grain structure of the steel as it is cold worked during the drawing of the shell is placed in a strained condition which must be relieved by heat treatment in order for the shell to satisfactorily function in the gun, extract with ease, and not split upon firing. It is possible that there is a partial recrystallization during this heat treatment. It is to be understood that the time of treatment depends on the material or precise alloy used and the temperature of the relief anneal and is not limited to that shown.

In Fig. 3 are shown the results of tests on cartridge cases of different metals treated in different manners. The force in pounds required to extract the cartridge from the chamber of the gun after it has been fired and the percentage of splits occurring are shown. A gilding metal case requires about 13 pounds extraction force when it is fired with a standard load, and a gilding metal case fired with a high velocity load requires in the vicinity of 32 pounds. The standard load gilding metal case is considered satisfactory.

A carbon steel case as drawn requires about 27 pounds extraction force after firing, and about 5% of those fired will have body splits. It is obvious that this is not a satisfactory case. When the carbon steel is relief annealed at 448° C. for one hour, no split shells will be found, but there will be an extraction force of 32 pounds required, which is too high an extraction force.

If an alloy steel be used of the analysis similar to that set forth below, there will be 57% of the cases split and 4½ pounds extraction force required. However, the same alloy steel when it

is relief annealed at 498° C. for one hour will give no split shells, and the extraction force required will be about 14 pounds, which is satisfactory for the high velocity loads. It is seen, therefore, that the relief annealed alloy steel gives results that are better than carbon steel as drawn or relief annealed, and is comparable to the gilding metal standard load fired characteristics.

- 10 Considerable strain is set up in the rim portion of the shell as it is formed, which tends to affect the sensitivity or the energy required to be directed against the rim of the shell in order to insure that the priming mixture will be ignited.
- 15 The sensitivity is increased by the relief annealing below the recrystallization temperature. In general, the higher the relief annealing temperature, the better will be the sensitivity characteristics of the shell, because the rim portion has the stresses relieved and becomes softer. A specific example of a satisfactory alloy steel is one having a composition of:

|           | Per cent |
|-----------|----------|
| Carbon    | 10       |
| Manganese | .50      |
| Nickel    | 1.50     |
| Chromium  | .75      |

Steels containing not over .50% carbon and, preferably, .10% carbon, containing any of the following elements, singly or in combination: chromium, cobalt, copper, manganese, molybdenum, nickel, phosphorus, silicon, titanium, vanadium in such quantities as to cause a substantial increase in the yield point will be satisfactory. As an example of this, the increase of from 35,000 pounds per square inch for carbon steel to 50,000 pounds per square inch for alloy steel before shaping without making the steel unworkable in the forming and pressing operations, will give satisfactory results.

As other examples, there may be cited a steel containing:

|        | Per cent |
|--------|----------|
| Carbon | .15      |
| Nickel | 1.50     |

or a steel of the following composition:

|           | Per cent |
|-----------|----------|
| Carbon    | .09      |
| Chromium  | .48      |
| Manganese | 1.47     |
| Silicon   | .54      |

It is to be understood, however, that these are merely specific examples and are not to be construed as limiting the invention thereto. Other alloying elements may also be employed within the steel.

The stress relieving heat treatment removes the internal stresses in the component.

In order to obtain the necessary characteristics for proper extraction and strength, particularly for high velocity loads, it has also been found possible by heat treatment of the components to obtain the correct strength in the finished component, as well as to secure this by means of alloying metals. Before the final draw, such as after the operation at Fig. 2—C, the component may be heated so that it is in the austenitic field, and then cooled at such a rate that the final structure is neither austenite nor pearlite, but is in a hardened transition phase between austenite and pearlite, being in the group which consists of martensite troostite, sorbite and bainite, and also includes these in their tempered form.

The succeeding drawing operation, such as to obtain the form shown in Fig. 2—D, will work-harden the metal, and the strength will be correspondingly greater than if the component had not been hardened by heat treatment before the drawing, due to the fact that the initial strength before work-hardening was increased by the heat treatment. The amount of the increase of strength, due to the work hardening, is greater than the increase of tensile strength by work hardening steel that has not been thus heated before the final draw, because it has been found that the fine dispersion of the carbides increases strength obtained by work-hardening over that obtained by work hardening of steel that does not have the carbides thus dispersed. The dispersion of the carbides may also be obtained by heating to the austenitic field and cooling in air, which is known as normalizing. The rate of increase of strength in cold shaping increases with the dispersion of the carbides. At this point, the component has more than sufficient strength, but it is so hard that it will not perform properly and would split in the chamber of the gun upon firing. It is necessary, therefore, to stress relieve the component, and such may be done by subjecting it to a temperature and for a time sufficient for this purpose, as has previously been pointed out. There will be a resultant loss in strength, but because the strength was sufficiently high after the final draw, the residual strength after the stress relieving treatment will be sufficient so that the shell will perform satisfactorily. In the stress relieving treatment, the component has been given the proper ductility to prevent splitting and also to give it the proper sensitivity. It is to be understood that it is merely necessary that the fine dispersion of the carbides be made before a final or last cold shaping takes place, and that if the drawing be done in one operation, that the single draw would be the same as the final draw.

As a specific example, a steel containing .22% carbon was treated by first cupping the blank, as at 2—B, following which it was annealed at a temperature in the vicinity of 620° C. so as to facilitate the succeeding drawing operation. It was then drawn to a form approximately as shown in Fig. 2—C. Following this, it was heated to about 980° C., which is in the austenitic field, and then quenched in oil. It was then tempered for one-half hour at about 590° C. At this point, the component has the carbides finely dispersed. The component was then drawn, placing it in the form similar to that of 2—D, and then cut off to the proper length and headed so as to be similar to that of Fig. 2—E. Following this, it was stress relieved at a temperature of about 450° C. for one hour, and the shell required less than about five pounds' extraction force and no splits occurred. As another example of treatment following the drawing operation of Fig. 2—C, the component may be normalized by heating to about 930° C. and allowed to cool so as to finely disperse the carbides, it not being quenched in oil, nor tempered, as in the previous example. Following the normalizing treatment, it was treated and shaped similar to that of the first example. The extraction force in this case was slightly higher than was the extraction force where the component was oil quenched and tempered.

In order to perform satisfactorily in the high velocity loads, it is desirable that the residual yield point strength of the completed component

be at least 90,000 pounds per square inch, and preferably around 110,000 pounds per square inch. The elongation should be at least the equivalent of 5% in 2", preferably about 10% or more, this being difficult to determine because the usual length of a shell, such as a .22 caliber, is shorter than 2". The Brinell hardness of the completed component should be at least 230, and preferably about 240.

It is to be understood, however, that these figures are examples of characteristics found to give satisfactory extraction and performance characteristics, and that they may vary.

It is apparent from the foregoing description that a new method and a new ammunition component have been produced that will be more economical to produce, and that will be satisfactory in their performance. The steel shells will not be subject to season cracking, and certain powders and priming materials may be used therein without difficulty. As this is believed to be the first time a satisfactory steel ammunition component and method of producing the same have been provided, it is not to be limited to the details and composition as shown herein, but is to be broadly construed as covering all equivalent devices and processes falling within the scope of the appended claims.

What is claimed is:

1. In the manufacture of cartridge cases from low carbon steel having a carbon content between about .09% and about .5% by drawing and annealing, the method comprising the steps of heating the case to the austenitic field, treating the case so as to obtain a hardened transition phase between pearlite and austenite, cold shaping the case, and then subjecting the cold shaped case to a stress relieving heat treatment, the hardening heat treatment and relief anneal being so coordinated that the increase in strength due to work hardening in the cold shaping will be sufficient so that the decrease in strength due to the stress relieving anneal will leave the required strength in the finished case.

2. In the manufacture of cartridge cases from low carbon steel having a carbon content between about .09% and about .5% by drawing and annealing, the method comprising the steps of heating the case to the austenitic field, treating the case so as to obtain a hardened transition phase between pearlite and austenite, cold shaping the case, and then heating to a temperature between about 300° and 550° C. for a period between about four hours and ten minutes, the hardening treatment and last mentioned heating being so coordinated that the increase in strength due to work hardening in the cold shaping will be sufficient so that the decrease in strength due to the stress relieving anneal will leave the required strength in the finished case.

3. In the manufacture of cartridge cases from low carbon steel having a carbon content between about .09% and about .5% by drawing and annealing, the method comprising the steps of normalizing said case to increase the rate of work hardenability and obtain a strength so coordinated with the relief anneal that the increase of strength due to work hardening in the final cold shaping will be sufficient so that the decrease of strength due to the stress relieving anneal will leave the required strength in the finished case, cold shaping the case, and then subjecting the cold shaped case to a stress relieving heat treatment.

CHARLES D. COXE.

CERTIFICATE OF CORRECTION.

Patent No. 2,341,264.

February 8, 1944.

CHARLES D. COXE.

It is hereby certified that error appears in the printed specification of the above numbered patent requiring correction as follows: Page 1, second column, line 28, for "deforation" read --deformation--; page 2, first column, line 14, for "of" read --or--; and that the said Letters Patent should be read with this correction therein that the same may conform to the record of the case in the Patent Office.

Signed and sealed this 18th day of April, A. D. 1944.

Leslie Frazer

(Seal)

Acting Commissioner of Patents.